

## UNITED STATES PATENT OFFICE

JOHN DE GIOVANNI, OF BROOKLYN, NEW YORK, ASSIGNOR TO POLYMET MANUFACTURING CORPORATION, OF NEW YORK, N. Y., A CORPORATION OF NEW YORK

## ELECTRIC MATERIAL AND PROCESS FOR MAKING SAME

No Drawing.

Application filed January 27, 1927. Serial No. 164,128.

This invention relates to electric materials and is directed to the provision of a novel conducting material adapted to serve as resistance elements and for the like purposes, 5 and a process for producing the same.

The increased use of electrical apparatus which has recently been stimulated particularly by the wide and general use of radio receiving apparatus has created a necessity 10 for a resistance material which will afford relatively high resistances without becoming too hot in operation. The heat developed in the ordinary resistance as now employed in the form of copper or German silver wire and 15 the like makes necessary special provision for effective heat radiation and even where such provision is made, the heated resistance element makes operation of the particular electrical apparatus dangerous as well as inefficient and uneconomical and very often results in the necessity of replacing parts or 20 discarding the unit.

Another disadvantage of the resistances now employed is that where coils of wire have 25 to be used to afford a high resistance, a large length of wire has to be used to give the desired amount of resistance, thus involving a comparatively high cost.

It is the object of this invention to provide 30 a conducting material which shall give effective resistance with efficiency in operation and comparatively little heating, and furthermore be economical in use, both as to the space occupied and the amount of material required to produce a given ohmic 35 quantity.

Other objects of this invention will in part be obvious and in part hereinafter pointed out.

40 In accomplishing these and other objects, I have availed myself of the well known fact that nearly all salts of metals are reduced more or less to a metallic state by the action of ultra violet light. Silver salts have been 45 found to be more sensitive than others in this connection. Thus silver bromide when subjected to ultra violet light will readily be reduced so as to leave a deposit of metallic silver. Briefly described, I provide a resistance material wherein a cheap mounting of

insulating material is employed as the body portion or base on which a metallic coating is formed which provides a thin conducting surface that affords the resistance to the electric current.

The following is an example of the carrying out of my invention: I make a solution of a silver salt such as silver nitrate and a solution of potassium bromide. The silver nitrate solution is then mixed thoroughly with a binder preferably in the form of an emulsion of some adhesive substance, such for example as gelatin. A sufficient quantity of the potassium bromide is then added to reduce the silver to silver bromide. There results a mass of silver bromide particles suspended in the gelatin emulsion. The base or mounting is then dipped in the solution and held therein so as to become impregnated therewith. It is then dried in any suitable manner under exposure of ordinary daylight, which reduces the bromide to some extent to metallic silver. The impregnated mounting is then immersed in an organic reducer such as paramido-phenol and sodium sulphite so as to completely reduce the bromide to the metallic silver. The material is then washed and dried.

For the mounting I preferably employ a cheap nonconducting material such as blotting paper which is sufficiently porous so as to become easily impregnated. There results from the treatment of this blotting paper as hereinbefore described, a flat material which is flexible and can be rolled up and cut as desired, having a fine coating of silver.

It will be seen that the material made in accordance with the foregoing description comprises a comparatively thick, non-conducting body portion on which is spread a very thin, metallic film of large superficial area which serves as the conductor for the current. I have found that this material while affording the resistance to the flow of the electric current will nevertheless be very little heated. More specifically, I have found, for example, that when a piece of this material, the ohmic resistance of which has been determined, is connected in series with a copper wire of the same resistance so that

55

60

65

70

75

80

85

90

95

100

the same current flows through both under the same E. M. F., the wire will get much hotter than the material, the latter remaining comparatively cool.

5 Other mounting materials and other metal coatings may of course be employed. Where a sufficiently porous material cannot be used, the impregnation may be effected under pressure.

10 The binder solution, like the mounting, should also be preferably of an adhesive substance which is non-conducting.

The invention has been described particularly with reference to the practical application of the material for electrical resistances.

15 It will of course be understood that it may serve other purposes for which electrical conducting materials are usually employed.

In addition to making up this material in 20 flat strips as will result from the particular illustration herein described, I contemplate making the material up also in the form of wire. For this purpose, the ordinary enamelled or cotton covered wire may be employed. The outside covering of the wire is 25 used for the backing and is impregnated in the same manner as above described. The copper wire itself is employed only to provide a core or base to give body to the material and 30 connection is made to the outside covering where electrical contact is had by means of the thin metallic layer.

It will thus be seen that there is provided 35 an article of manufacture and process in which the several objects of this invention are achieved, and which are well adapted to meet the conditions of practical use.

Having thus described my invention, I 40 claim as new and desire to secure by Letters Patent:—

1. The herein described process for making materials of the character described consisting in impregnating a conducting member having a central metallic wire and a covering of insulating material with a solution of 45 a silver salt and reducing said salt.

2. The herein described process for making materials of the character described consisting in mixing an emulsion of silver nitrate 50 with a solution of potassium bromide, of dipping a conductor cable having an outer cover of porous non-conducting material into said mixture until said cover is impregnated, of drying the resulting material in daylight, of 55 then impregnating the said material in para-mido phenol and sodium sulphite and of washing and drying the resulting product.

In testimony whereof I affix my signature.  
JOHN DE GIOVANNI.